

# UNITED STATES PATENT OFFICE.

EDITH L. SNYDER, OF JOHNSTOWN, PENNSYLVANIA.

## OIL WATER-COLOR PAINT.

1,327,928.

Specification of Letters Patent.

Patented Jan. 13, 1920.

No Drawing.

Application filed August 10, 1917. Serial No. 185,541.

*To all whom it may concern:*

Be it known that I, EDITH L. SNYDER, a citizen of the United States, and a resident of Johnstown, in the county of Cambria and State of Pennsylvania, have invented 5 certain new and useful Improvements in Oil Water-Color Paint, of which the following is a specification.

My invention relates to oil water color 10 paint and has for its purpose the provision of a paint having a wide range of usefulness containing oil and having many of the advantages of oil paint, while applicable by means of water as a vehicle. Most water 15 color paints wash off readily so that attempting to paint over with another color a color already laid on washes it off or mingles the two and precludes obtaining effects and pursuing methods usual with oil paints. 20 An important characteristic of my paint, on the contrary, is that it is waterproof on drying and, as it dries comparatively rapidly, painting with one color over 25 another without disturbing it presents no difficulty. Since this paint of mine is suited not only for rough work but also for the finest water color painting, the importance of this will be appreciated since it makes possible the handling of water color painting 30 in much the same way as oil painting and removes hampering limitations.

My paint is especially effective for scene painting and for decorating and may be used for all classes of work under these 35 heads except for sizing, that is, for shadow work, commonly known as "dirty work," for making the sketch and for finishing. My paint as herein described is a paste which remains soft or moist in tubes and jars, and 40 to which water may be added to make it sufficiently fluid to be applied with large brushes for the rougher work, or which may be applied by wetting small brushes as in fine water color work. It will be understood 45 that I may use any desired pigment or pigments just as in the usual water colors.

My invention thus consists of the oil water color paint described in the specification and set forth in the appended claims.

50 The ingredients I employ, in addition to the coloring matter, are glycerin, white of egg, drying oil, copal varnish and glue. I am accustomed to use both linseed oil and pale, or thin drying oil, of which also linseed oil is the basis, and liquid glue. The vehicle of the copal varnish which I have 55

employed is pure linseed oil and it is so light in color as to be known as "white copal varnish." This makes it suitable for even the lightest colors, which may also be said of 60 the "pale drying oil." It will be understood that I may use in lieu of any of the above ingredients any materials which are or may be found to be the equivalents thereof in my 65 composition.

The proportions of the various ingredients which have proved to be suitable will be illustrated herein by examples, but it will of course be understood by those familiar with this art, that proportions may be varied 70 within a considerable range with different pigments and according to the special requirements or individual taste of the user. For instance, for a comparatively coarse heavy pigment, such as burnt sienna, more 75 glycerin would be required, while less would be needed for a vegetable pigment, such as rose madder.

I make up my paint cold and, if mixing it by hand, prefer to mix the pigment in the 80 form of a powder with glycerin to a thick paste and then add each ingredient separately as in formula. If the mixing is done by machine all the ingredients may be placed in the machine together. The paste, when 85 the mixing is finished, should be cut short, that is when a small portion is removed by a palette knife, the cut should be sharp and clean. The effect of putting in too much of the white of egg is to make the paste too thin 90 and fluffy and to lessen its adhesive properties. Too much glycerin also makes the paste too thin.

Without attempting to designate every function of each ingredient or its precise relation in the composition, I may state that 95 my understanding of the part played by the various ingredients in my paint is generally speaking as follows:

The glycerin assists in making up the 100 paint body and keeps the composition soft or moist, preventing it from drying up and getting hard when used in paste form. The white of egg and the liquid glue are adhesive binders. The white of egg makes 105 the paste short and, since it works transparent, assists the glycerin effectively. The linseed oil gives body and it, as well as the drying oil, is a drier, the latter accelerating this effect, and both these oils play a part in 110 making the paint waterproof on drying and in adapting it to uses and results which

may be secured with ordinary oil paint. The copal varnish acting in connection with the oils is believed to be the agent which makes the paint waterproof on drying, and in addition to furnishing adhesive properties, the glue, and perhaps also the glycerin and the white of egg, assists in giving the composition the characteristics which enable it to be used with water as the vehicle. If the paint will not work with water more glue should be added.

It will be understood, of course, that my paint may be mixed in any quantity desired, although the formulas which I am about to give are for relatively small quantities which may be mixed by hand. It being obviously impossible in this specification to give for all the various pigments formulas exactly adapted to each, I will confine myself to two characteristic formulas: one for zinc white and the other for burnt sienna. These are as follows:

*Zinc white.*

|    |                         |       |
|----|-------------------------|-------|
| 25 | Zinc white              | 1 lb. |
|    | Glycerin                | 4 oz. |
|    | White of egg            | 2 oz. |
|    | Linseed oil             | 4 oz. |
| 30 | Pale or thin drying oil | 4 oz. |
|    | Copal varnish           | 4 oz. |
|    | Liquid glue             | 4 oz. |

*Burnt sienna.*

|    |                         |        |
|----|-------------------------|--------|
| 35 | Burnt sienna            | 1 lb.  |
|    | Glycerin                | 10 oz. |
|    | White of egg            | 2 oz.  |
|    | Linseed oil             | 4 oz.  |
| 40 | Pale or thin drying oil | 4 oz.  |
|    | Copal varnish           | 4 oz.  |
|    | Liquid glue             | 4 oz.  |

As to these formulas, it is to be noted that the proportionate amounts given are those found to give the best results, but they are not to be understood as precluding reasonable variations. The zinc white for-

50 mula may be regarded as a sort of standard, since it is applicable to other pigments of substantially the same weight and fineness and may be modified in either direction for lighter and finer or heavier and coarser pigments. For the former relatively less and for the latter relatively more glycerin would be required. It is believed that one familiar with the art would, in the light of 55 what has been said, have no difficulty in determining the proper proportions for any given pigment.

What I claim as my invention is:

1. Oil water color paint containing coloring matter, glycerin, white of egg, drying oil, copal varnish, and glue applicable by means of water as a vehicle, and which is waterproof on drying.

2. Oil water color paint containing coloring matter, glycerin, white of egg, linseed oil, a drier, copal varnish, and liquid glue.

3. Oil water color paint containing coloring matter, glycerin, white of egg, linseed oil, thin drying oil, copal varnish and liquid glue, which when in paste form cuts short, 70 is applicable by means of water as a vehicle and is waterproof on drying.

4. Oil water color paint containing coloring matter, glycerin, white of egg, linseed oil, thin drying oil, copal varnish and liquid glue, in approximately the proportions described, the said paint being suitable for both rough and fine work.

5. Oil water color paint containing in approximately 80 the proportions indicated by the amounts stated: coloring matter one pound; glycerin four to ten ounces; white of egg two ounces; linseed oil four ounces; thin drying oil four ounces; copal varnish 85 four ounces, and liquid glue four ounces.

In testimony whereof I affix my signature in presence of two witnesses.

EDITH L. SNYDER.

Witnesses:

MARY MARTHA SCHETTIG,  
ALEX N. HART.